

Feb. 16, 1932.

L. E. POWER

1,845,811

RESISTOR UNIT AND METHOD OF FORMING THE SAME

Filed June 8, 1927

*Fig. 1.*



*Fig. 2.*



*Fig. 3.*



*Inventor:*

Laurence E. Power

*By: Ira Milton Jones  
Attorney*

## UNITED STATES PATENT OFFICE

LAURENCE E. POWER, OF MILWAUKEE, WISCONSIN, ASSIGNOR, BY MESNE ASSIGNMENTS, TO ALLEN-BRADLEY COMPANY, OF MILWAUKEE, WISCONSIN, A CORPORATION OF WISCONSIN

## RESISTOR UNIT AND METHOD OF FORMING THE SAME

Application filed June 8, 1927. Serial No. 197,367.

This invention relates to certain new and useful improvements in resistor units and method of forming the same and refers especially to units designed for use in radio receiver circuits and the like.

It is highly desirable that resistor units utilized in radio receiver circuits and the like have a predetermined resistance value, depending upon the particular circuit, which value must be substantially correct within a slight latitude and heretofore it has been impossible to produce units of predetermined resistance values with any degree of accuracy except by adjusting them in the manner illustrated in the copending application of Lynde Bradley, Serial No. 53,570.

However, this manner of producing resistor units, while efficient, is objectionable in that it involves considerable handling of the units and the attendant labor expense, and, therefore, it is an object of this invention to provide an improved method of producing resistor units whereby the units may be made in quantities having a predetermined resistance value without requiring unnecessary handling of the units.

Another object of this invention resides in the provision of an improved method of forming resistor units in which the ingredients are such as to permit the production of resistance units of predetermined value by controlling the proportions of the ingredients, whereby the necessity of adjusting the units after formation is eliminated.

Another object of this invention resides in the provision of an improved resistor unit having a carbon black, such as gas black or lamp black, incorporated therein as a conductor together with asbestos fibre and clay or the like, as a filler, and a phenol condensation product as a binder.

A further object of this invention resides in the provision of an improved method of forming resistor units having a predetermined resistance value which consists in thoroughly mixing gas or lamp black with a filler including asbestos and a binder, preferably phenol resin, reducing the mixed ingredients to a powder, blending stock powders with the mixture to increase or decrease the

percentages of conductivity of the materials to thus produce predetermined conductivities and forming the blended powder into the finished units.

It is a still further object of this invention to provide an improved method of forming resistor units by first molding the ingredients sufficient for one unit into a slug or bar and in forming the unit from the slug or bar.

With the above and other objects in view which will appear as the description proceeds, my invention resides in the novel construction, combination and arrangement of parts substantially as hereinafter described and more particularly defined by the appended claims, it being understood that such changes in the precise embodiment of the herein disclosed invention may be made as come within the scope of the claims.

In the accompanying drawings, I have illustrated one complete example of the physical embodiment of my invention constructed according to the best mode I have so far devised for the practical application of the principles thereof, and in which:

Figure 1 is a side elevational view of the slug or bar into which the ingredients of a resistor are initially formed;

Figure 2 is a vertical sectional view through a forming mold illustrating the molding of the slug to form the finished unit, and

Figure 3 is a side elevational view of a completed resistor unit.

Referring to the drawings, the numeral 5 designates a complete resistor unit having a body 6 composed of a conductor, a filler and a binder, as later described, and provided with end cap or terminal members 7, the terminal members 7 providing means for mounting the unit within an electrical circuit, not shown.

In radio circuits, it is of utmost importance that the units have definite resistance values and great difficulty has been experienced in obtaining any definite value, the most successful method now in use being that described in the copending application referred to. The method of setting or adjusting the resistance value of the units by "shooting", i. e., subjecting them to the influence of an

electrical current having the capacity to reduce their resistance value, is open to the serious objection that the unit must be handled considerably in manufacture, thus adding 5 to the labor cost. This objectionable feature is overcome and a resistance unit of any desired resistance value is produced by controlling the proportions of the ingredients entering therein.

10 It has been found from practice that the following mixtures when molded into a resistance unit produce units of the values noted:

15 Resistor units of approximately one million (1,000,000) ohms:

Conductor, such as gas or lamp black 25%

Filler, such as asbestos fibre and clay 28%

Binder, such as a phenol condensation

20 product 47%

Resistance units of approximately forty million (40,000,000) ohms:

Conductor, such as gas or lamp black 18%

25 Filler, such as asbestos fibre or asbestos fibre and clay 37%

Binder, such as phenol condensation product 45%

30 The above are merely examples of the combinations used and should it be desired to obtain values other than those mentioned above, the mixtures are planned accordingly.

To produce a batch of mixture for resistance units, phenol resin is first made from 35 phenol formaldehyde, ammonia, etc. which is cured to a point where it is hard at the ordinary room temperature and soft when heated. This hardened phenol resin is then ground to a powder and the other materials 40 such as fillers and conductors are mixed therewith in a ball mill.

The ingredients are then further mixed 45 hot on rollers, such as rubber calenders, the heat being obtained by the dissipation of energy in rolling, the resultant product being a sheet of the commingled ingredients.

The sheet is then broken up and ground 50 to a powder, which forms the base for the resistance units and the proportion of ingredients thereof produces a unit of the maximum resistance value, and assuming the maximum resistance desired is forty million ohms, the proportions are as mentioned above in the second example. This stock mixture 55 is then further blended with other mixtures of the same ingredients to vary the proportions according to the conductivities required, the blended mixture being formed into sticks or slugs 8, preferably by an automatic tablet machine, not shown.

60 Each stick or slug is then placed in a mold 9 and subjected to a pressure of roughly 160 tons per square inch, through a plunger or pin 10. The units are then baked or treated under an air pressure of roughly two hundred

pounds per square inch at a temperature of four hundred degrees (400°) Fahrenheit. The units are then complete and the end terminals or caps 7 are pressed on the ends to provide means for incorporating the units 70 within an electrical circuit and it will be apparent that the end terminals may be dispensed with, if desired, as illustrated in my copending application Serial No. 197,882.

From the foregoing description taken in 75 connection with the accompanying drawings, it will be readily apparent to those skilled in the art to which an invention of the character described appertains that I provide a novel and improved resistor unit and method 80 of forming the same which is capable of production at a lower cost and which is very efficient in operation.

What I claim as my invention is:

1. A resistor unit having approximately 85 one million ohms capacity, consisting of approximately twenty-five per cent carbon black, approximately fourteen per cent asbestos fibre, approximately fourteen per cent clay, and approximately forty-seven per 90 cent phenol condensation product.

2. The herein-described method of forming a resistor unit which consists in thoroughly commingling carbon black, asbestos fibre and a phenol condensation product, in preforming the ingredients into a stick capable of maintaining its own form, and in finally forming the unit from the stick.

In testimony whereof I have hereunto affixed my signature.

LAURENCE E. POWER.

105

110

115

120

125

130